

## UNITED STATES PATENT OFFICE.

JOHN J. GANNON, LOUIS W. MAHLE, AND FRED B. WELLS, OF RITTMAN, OHIO, AS  
SIGNORS TO THE OHIO BOXBOARD COMPANY, OF CLEVELAND, OHIO. A CORPORA-  
TION OF OHIO.

## PAPER MAKING.

No Drawing.

Application filed April 6, 1926. Serial No. 21,221.

In packaging certain merchandise, such as lard, butter, and other greases and fats, it is desirable to have a container which is made of a grease-proof material; also, in packaging materials, which are, from their inherent nature, apt to absorb moisture from the atmosphere, it is advisable to provide a container which is made of a moisture-proof material; it is also advisable, in packaging materials which deteriorate in a humid or moist atmosphere, and which are, moreover, of a greasy or oily nature, such as nuts and soaps, to provide a container which is both grease-proof and moisture-proof; and it is the object of our invention to produce a material, in the nature of a boxboard, which is grease-proof, or both grease-proof and moisture-proof.

Various types of papers, and of boxboard and cardboard, have been produced for providing a material suitable for the construction of grease-proof, moisture-proof, or both grease-proof and moisture-proof containers. Some of such materials comprise a base of ordinary paper, or cardboard or boxboard, to one surface of which is affixed, by pasting or cementing, a sheet of ordinary paraffine or wax or other suitable pergameneous paper. This type of material is more or less expensive to manufacture, and must, necessarily therefore, be sold at a rather high price, due to the fact that in its production at least three distinct operations are necessary, namely, production of the paper, cardboard or boxboard, production of the moisture-proof or grease-proof paper, and combination of these two to form the finished, laminated material.

Moisture-proof material has been produced also by pasting together two or more sheets of paper, cardboard or boxboard with asphalt or water glass (sodium silicate) or the like as the adhesive. This type of material, although effective to prevent penetration of water or moisture through it, is also relatively expensive to manufacture.

As distinguished from papers and boards of the types last above mentioned, our invention contemplates the incorporation with a boxboard of ordinary type, of a grease-proof or both grease-proof and moisture-proof material integrally with the main body of the boxboard in a single paper-making operation.

The invention consists in a method of making paper, such as cardboard, boxboard or the like, comprising, essentially, combining with the body-forming portion or filler of the paper during the paper-making operation of the paper machine, a layer of grease-proof material, or both grease-proof and moisture-proof material, as an integral part of the sheet of paper, as we will proceed now to explain and finally claim.

Boxboards produced in accordance with our invention will ordinarily comprise a filler or body-forming portion of a thickness suitable to provide the strength desired in the finished board, a back, and a layer or coating of the grease-proof or both grease-proof and moisture-proof material, preferably formed as a surface layer or coating on the side or face of the filler opposite to that to which the back is applied, the whole being produced at a single operation. However, the arrangement of the component parts of the board may, if desired, be varied to suit certain predetermined requirements.

The stock for forming the filler is produced in the ordinary manner by working old newspapers and the like in an ordinary beater, and the stock for the back is similarly produced, but has added to it agents or materials for making it of a higher grade and better color than the filler.

The grease-proof stock, for forming the layer or coating, is produced in the following manner:—Pure sulphite pulp is worked in a beater having, as distinguished from the ordinary beater, a roll of stone, preferably of basalt lava, which, in its operation upon the stock, crushes the fibers of the sulphite pulp instead of cutting them, as distinguished from the operation of the ordinary beater having a roll with steel fly bars. This crushing of the fibers of the stock, the hydration of same incident to the beating action, and the mechanical working of the stock by the stone roll, so breaks up and macerates the sulphite pulp that it forms a grease-proof product. This operation and the stock used (sulphite pulp) are the same as are employed in the manufacture of one well-known type of pergameneous paper hereinabove referred to.

The working of the sulphite pulp in a beater having a stone roll, as described, has been found to produce a change in the stock,

whereby it is rendered grease-proof, or 5 grease-repellent, which is not produced in the same stock by working it in the ordinary beater wherein the ordinary roll with steel fly bars is used. It has been found possible to produce the same change in sulphite pulp stock by working it in a ball mill, or with a mortar and pestle.

This stock, formed from pure sulphite 10 pulp, is, as stated, grease-proof or grease-repellent, and is therefore suitable for incorporation with filler stock to form a grease-proof paper or board. However, if it is desired to produce a paper or board 15 which is both grease-proof or grease-repellent and water or moisture-proof, it is necessary to add to the sulphite pulp stock, preferably during the beating process, a suitable wax, resin size, or other sizing 20 agent, which is miscible with the sulphite pulp stock. In the case of the addition to the stock of a wax, such as paraffine wax, it will be found advisable, in order to produce 25 a homogeneous and inseparable mixture of the wax and the sulphite pulp stock, first to prepare an emulsion of the wax, and then add such emulsion to the sulphite pulp stock.

In forming the paper or board of our 30 invention, we use, preferably, a cylinder machine (although our material may be produced by the Fourdrinier process), and after the stock for the various component parts of the paper, above enumerated, has 35 been suitably beaten, digested and washed, it is deposited by the cylinders of the machine (any number of cylinders being used to produce the required thickness of paper) to form the sheet. No particular order of 40 deposition of the various paper stocks in the formation of the sheet is essential, but we have found that the best results are obtained either by depositing first the pure sulphite pulp stock, then the filler, and then 45 the back, or first the back, then the filler, and then the pure sulphite pulp stock. The sheet thus formed is thereafter squeezed, dried and calendered in the usual way.

Paper or board manufacturers would 50 probably say that it would be impossible to incorporate pure sulphite pulp stock treated to form a grease-proof product, as above described, in a board, for the reason that, being a much slower stock, (that is, one 55 through which water is not easily expressed) than stock generally used in board manufacturing, the water could not be driven from the stock effectively, and the finished sheet would contain "blows" or 60 bubbles between the sulphite pulp stock layer or coating and the filler or other layer next adjacent to it; but we have found that all of the water may be driven off in a direction away from the sulphite pulp stock layer, and a sheet produced which is en-

tirely free from "blows", bubbles or other imperfections.

We have hereinbefore described our invention as applied to a paper or boxboard suitable for the formation of containers for 70 various articles of merchandise, and in thus describing the invention, we have intended that it should be understood that the paper or boxboard is used alone for the formation of such containers and without any 75 strengthening or stiffening backing. However, the paper or board produced in accordance with our invention may be put to a variety of uses. It may be used, for example, as a liner or back for corrugated board or 80 fiber board, or it may be incorporated in what is known as pasted board with asphalt, water glass, glue, or the like, as the adhesive, and will, when thus used, produce a material which, in addition to its other ordinary characteristics, is grease-proof or grease-repellent or both grease-proof and moisture or water-proof.

Reference is made to our copending application for patent for improvement in 90 paper, filed April 6, 1925, Serial No. 21,222 which covers the product produced by the process hereinbefore described.

The invention is susceptible of various modifications within the scope of the following claims.

What we claim is:—

1. A process of making paper, which consists in depositing a layer of pergameneous material, depositing thereon a layer of filler material, and thereafter expressing the surplus water from the thus combined layers in a direction away from the layer of pergameneous material and through the layer of 100 filler material.

2. A process of making paper, which consists in depositing a layer of pergameneous material, depositing thereon a layer of filler material, and thereafter expressing the surplus water from the thus combined layers in a direction away from the layer of pergameneous material and through the layer of 110 filler material and drying and calendering said material to form an integral sheet.

3. A process of making paper, which consists in depositing a layer of pergameneous material, depositing thereon a layer of filler material, depositing upon said filler material a layer of back material, and thereafter expressing the surplus water from the thus 120 combined layers in a direction away from said pergameneous layer and through said filler and back to form an integral sheet.

4. A process of making paper, which consists in depositing a layer of pergameneous material, depositing thereon a layer of filler material, depositing upon said filler material a layer of back material, and thereafter expressing the surplus water from the thus 125 combined layers in a direction away from

said pergameneous layer and through said filler and back and drying and calendering said material to form an integral sheet.

5. A process of making paper, which consists in depositing a layer of pergameneous paper stock comprising sulphite pulp stock prepared to form a grease-proof material, depositing thereon paper stock for forming the body of the paper, and thereafter expressing the surplus moisture from the

thus combined stock in a direction away from the layer of pergameneous stock and through the body-forming stock.

In testimony whereof we have hereunto set our hands this third day of April A. D. 1925.

JOHN J. GANNON.  
LOUIS W. MAHLE.  
FRED B. WELLS.

said pergameneous layer and through said filler and back and drying and calendering said material to form an integral sheet.

5. A process of making paper, which consists in depositing a layer of pergameneous paper stock comprising sulphite pulp stock prepared to form a grease-proof material, depositing thereon paper stock for forming the body of the paper, and thereafter <sup>10</sup> pressing the surplus moisture from the

thus combined stock in a direction away from the layer of pergameneous stock and through the body-forming stock.

In testimony whereof we have hereunto set our hands this third day of April A. D. 1925.

JOHN J. GANNON.  
LOUIS W. MAHLE.  
FRED B. WELLS.

**Certificate of Correction.**

It is hereby certified that in Letters Patent No. 1,606,162, granted November 9, 1926, upon the application of John J. Gannon, Louis W. Mahle, and Fred B. Wells, of Rittman, Ohio, for an improvement in "Paper Making," an error appears in the printed specification requiring correction as follows: Page 1, line 105, strike out the words "hereinabove referred to"; and that the said Letters Patent should be read with this correction therein that the same may conform to the record of the case in the Patent Office.

Signed and sealed this 21st day of December, A. D. 1926.

[SEAL.]

M. J. MOORE,  
*Acting Commissioner of Patents.*

**Certificate of Correction.**

It is hereby certified that in Letters Patent No. 1,606,162, granted November 9, 1926, upon the application of John J. Gannon, Louis W. Mahle, and Fred B. Wells, of Rittman, Ohio, for an improvement in "Paper Making," an error appears in the printed specification requiring correction as follows: Page 1, line 105, strike out the words "hereinabove referred to"; and that the said Letters Patent should be read with this correction therein that the same may conform to the record of the case in the Patent Office.

Signed and sealed this 21st day of December, A. D. 1926.

[**SEAL.**]

**M. J. MOORE,**  
*Acting Commissioner of Patents.*